

Dec. 22, 1931.

C. E. MAYNARD

1,837,461

MARKING RUBBERIZED MATERIAL

Original Filed June 2, 1928



INVENTOR.

Charles Edgar Maynard.

BY

Charles E. Maynard

ATTORNEY.

## UNITED STATES PATENT OFFICE

CHARLES EDGAR MAYNARD, OF NORTHAMPTON, MASSACHUSETTS, ASSIGNOR TO THE FISK RUBBER COMPANY, OF CHICOPEE FALLS, MASSACHUSETTS, A CORPORATION OF MASSACHUSETTS

## MARKING RUBBERIZED MATERIAL

Original application filed June 2, 1928, Serial No. 282,322. Divided and this application filed September 11, 1929. Serial No. 391,853.

My invention relates to a method of marking continuous sheets of material and more particularly to a method for marking continuous sheets of rubberized cord or woven fabric such as is used in the manufacture of pneumatic tires. It has for one object the provision of a marking which may be imprinted on both sides of rubberized material and which without damaging the material and without the use of any marking agent will be easily distinguishable. Other objects will be apparent from the specification and claims.

The marking of rubberized cord or fabric stock for use in pneumatic tires has, up to the present, as far as applicant is aware, been a problem which has never been satisfactorily solved. The large production of the many grades of pneumatic tires now manufactured necessarily demands many grades of rubberized cord or fabric stock used in their manufacture. As it is very difficult to distinguish by appearance between the different grades of rubberized stock, it is advantageous to use some identifying means as it is calendered. Marking crayon was tried but found unsatisfactory as it introduces foreign matter into the finished tire, thus weakening its construction. Rubber cement has also been used and found objectionable due to the maintenance necessary and the relatively high cost of the materials used. My invention successfully overcomes all of these objections. In the attached drawings I have disclosed one manner of carrying out my method, the mechanism shown being claimed in my co-pending application, Patent No. 1,748,300, dated February 25, 1930, of which application the present is a division.

Fig. 1 is a perspective view of my invention, marking material coming from calender rolls;

Fig. 2 is a sectional view of one of the

marking roll supporting and positioning members;

Fig. 3 is a sectional view of the marking rolls;

Fig. 4 is a partial view taken on line 4—4 of Fig. 1 showing the locking bar; and

Fig. 5 is a view of a piece of material showing the identifying marks on both sides.

As indicated on the drawings, 10 represents a frame on which are mounted bearings 11 supporting a shaft 12 (Fig. 1). Keyed to the shaft 12 are two wheels 13 (Fig. 2) each having eight equally spaced radial guideways 14 and bolted on side plates 15. Around the periphery of wheel 13 are bolted indexing blocks 16. Confined in the radial guideways 14 by ball bearings 17 are marking rollers 18 which bear spacing collars 19 and marking dies 20 (Figs. 2 and 3) the latter being bolted to the rolls 18 by bolts 21 at different angles as shown in Fig. 1. For clearness only two such marking rollers are shown in the drawings but it will be obvious that six more, each with different marking dies 20, may be added by simply removing the correct indexing blocks 16, inserting the marking rollers and rebolting the indexing blocks.

Positioned below the marking rollers 18 and in the same vertical plane as shaft 12 is a roller 22 supported by bearings 23 to the frame 10 and over which travels the rubberized stock 24 from calender rolls 25. Linked to the bearings 11 by links 26 is a locking bar 27 (Fig. 4) kept in the correct vertical alignment by guiding slots in the extensions 28 of bearings 11. When the locking bar 27 is in the full line position shown in Fig. 4 it engages slots 29 in the uppermost indexing block 16 on each wheel 13 to position the diametrically opposite marking roller 18 in operating relation with the roller 22 as shown in Fig. 2. Any of the other marking rollers may be brought to this position by raising the locking bar 27 to the dotted line position shown in Fig. 4 and rotating the

60

65

70

75

80

85

90

95

wheels 13 to the correct indexing blocks 16.

As is shown in Fig. 2 the spacing collars 19 on the marking roller 18 rest on roll 22 and the ball bearing 17 engages the guideways 14 to prevent any horizontal movement but to allow a free vertical movement of the marking roller 18 thus giving the latter a floating roll action and, as the roll 22 is rotated by the stock 24, the spacing collars 19 will rotate the marking roller in the opposite direction (see Fig. 3).

The faces of the marking dies 20 are kept at a constant separation from the roll 22 by the spacing collars 19 (see Fig. 3) but as the separation is less than the thickness of the rubberized stock 24 the marking dies 20 produce an impression 30 on each side of the stock 24 as shown in Figs. 3 and 5. The weight of the combined marking roller 18, spacing collar 19, etc., is enough to overcome the resistance of the warm rubber so that the spacing collar 19 engages the roll 22 at all times.

The separation between the face of the marking dies 20 and the roll 22 is governed by the dimensions of the spacing collars 19 and has been found from experiment to be critical in so much as too little separation may permit the dies to cut the imbedded cords 31 and too great a separation will not produce a satisfactory marking. Following is a typical example with a roll weighing approximately 120 pounds:

|                                            |      |     |
|--------------------------------------------|------|-----|
| Average thickness of stock                 | .050 | 100 |
| Depth of compression needed for imprinting | .033 |     |

|                                          |      |     |
|------------------------------------------|------|-----|
| Separation between marking dies and roll | .017 | 105 |
|------------------------------------------|------|-----|

The warm rubber is in a condition to flow sufficiently easily to be displaced by the pressure of the die and this displacement takes place, as shown in Fig. 3, on both sides of the material if both sides are coated. Preferably the spacing of the dies from roll 22 is such that, assuming the material to be a cord fabric, a relatively thin film of rubber is left over the cords at the points of impression with the result that the lines of the cords show sufficiently to give the marking a characteristic lined appearance easily distinguishable from the relatively smooth surrounding surface. This lined effect is indicated in Fig. 5. When the coated material is a woven fabric as distinguished from cord fabric the marking shows the characteristic weave of the material. It will be understood that no rubber is removed and that the marking in no way harms the material.

Having thus described my invention, I claim:

1. The method of marking rubber coated material which comprises displacing the rubber coating while in a warm condition in a

predetermined pattern and to a depth sufficient to impart to the portion so treated the characteristic appearance of the underlying material without completely uncovering the material.

2. The method of marking rubber coated materials which comprises applying pressure to the rubber coating while in a plastic condition in a predetermined pattern to impart to the portion so treated the characteristic appearance of the underlying material without completely uncovering the material.

CHARLES EDGAR MAYNARD.

70

75

80

85

90

95

100

105

110

115

120

125

130